

Aug. 6, 1940.

R. WEINGAND ET AL

2,210,436

PROCESS FOR MAKING TUBING AND THE PRODUCT SO PRODUCED

Filed Oct. 27, 1937



Fig. 1.

Fig. 2.

Fig. 3.



INVENTORS  
 RICHARD WEINGAND  
 GUNTHER BRUMMACH  
 BY *Worth Wade*  
 ATTORNEY

## UNITED STATES PATENT OFFICE

2,210,436

PROCESS FOR MAKING TUBING AND THE  
PRODUCT SO PRODUCEDRichard Weinsard and Günther Brummeck,  
Ebersle, GermanyApplication October 27, 1937, Serial No. 171,276  
In Germany October 28, 1938

## 8 Claims. (Cl. 99—176)

The invention relates in general to tubing and, in particular, to tubing adapted for use as artificial sausage casings, and to correlated improvements designed to enhance the strength and durability of such tubing.

It is known to make tubing to be used, for example, as sausage casings, by coating or impregnating a strip of paper of suitable width with an albuminous substance, e. g., gelatine in solution, and thereafter pasting the edges of the treated strip of paper together to form a tube. This method, however, fails to produce a seam that will not readily tear or rupture because the edges are stuck together only after the paper has been coated with the albuminous substance. The reason for this lies in the fact that the bond formed by two layers of gelatine is weaker than that formed between paper and gelatine.

The general object of the invention is to provide a coated paper tubing having a seam that is strongly resistant to tearing or rupture.

It is a specific object of the invention to provide a sausage casing from fibrous sheet materials having a seam which will not become weakened during the soaking of the casing prior to stuffing and which will be highly resistant to rupture during stuffing, curing and cooking of the sausage.

It is a further object of the invention to provide a process for making sausage casings simulating natural casings from fibrous sheet materials in a simple, continuous and economical manner.

Other objects of the invention will in part be obvious and will in part appear hereinafter.

In the practice of the invention, a sheet of fibrous material is formed into a tube having a seam formed with a water-insoluble, non-fusible adhesive applied directly to the fibrous material, and thereafter the tube is treated by coating and/or impregnating with a water-swelling film-forming plastic material. The product is a tubing adapted for use as a sausage casing and characterized by having a seam which will not weaken during soaking of the tubing preparatory to stuffing or in any of the operations in the manufacture of sausages therewith.

The invention accordingly comprises the several steps and relation of one or more of such steps with respect to each of the others, and the article possessing the features, properties, and the relation of elements, which are exemplified in the following detailed disclosure, and the scope of the invention will be indicated in the claims.

For a more complete understanding of the nature and objects of the invention, reference should be had to the accompanying drawing in which:

Fig. 1 is a diagrammatical representation of

an apparatus for performing one embodiment of the process of the invention;

Fig. 2 is a perspective view of one embodiment of the article of the invention; and

Fig. 3 is a cross-sectional view of the article of Fig. 2.

For the fibrous sheet material there may be employed a suitable paper formed preferably of long vegetable fibres such, for example, as a paper formed of manila, mitsuma, kodzu and gampi plants and the like. The paper sheet is preferably one in which the fibres are non-oriented such, for example, as a sheet formed on a paper machine of the cylinder-sieve type. The thickness of the sheet may be varied in accordance with the size of tubing, having regard for the stuffing pressures employed in sausage manufacture and the weight of the sausage meat. Preferably a thin paper of the Yoshino or Japan type is employed, a sheet having a weight of about 40 grams per square meter being suitable.

It has now been found that it makes a difference what kind of adhesive is used to form the seam of the paper tubing prior to coating or impregnating with the film-forming material. If one uses, for example, the usual paper pastes, such as starch or gum arabic, such pastes will dissolve, partly or altogether, when the paper tubing is treated with the film-forming material in solution, because pastes of this type are extremely water-soluble and water-swelling. This disadvantage is particularly apparent when aqueous solutions of high temperature are used for coating the tubing. This difficulty can be successfully obviated if the edges of the paper sheet are united with an adhesive which is non-swelling and insoluble in water and unaffected by the temperatures used in the process of fabricating the tubing or in curing and cooking sausage. A suitable adhesive is a hydrophobic colloidal substance such as a natural or synthetic resin, a water-insoluble cellulose ester, cellulose ether, or an albuminous substance such as gelatine which has been insolubilized and rendered non-swelling by a suitable hardening agent such as formaldehyde, a chromate or the like.

For coating and/or impregnating the paper tubing there is employed a suitable hydrophilic organic film-forming substance capable of being transformed into a hydrophilic substance which is insoluble in water, but which swells therein and is non-fusible at the temperatures used in the cooking and curing of sausages. Suitable film-forming substances are the water-swelling colloids such as gelatine, casein and alkali-soluble or water-soluble cellulose ethers such, for example, as an oxy- or hydroxy alkyl cellulose ether, cellulose hydrate which may be regenerated from viscose or precipitated from solutions of cellulose in inorganic salts, ammonia or or-

ganic bases. The film-forming substance may be applied on the outside only of the tubing but is preferably applied both inside and outside the tubing. It is desirable to employ hydrophilic, i. e., water-swelling substances for the coating and/or impregnating of the tubing because such substances swell in water during the soaking of the tubing preparatory to stuffing and thus enable the tubing to expand somewhat during stuffing. During the curing of the sausage, the casing tends to dry out and the hydrophilic substance will shrink to a substantial extent and bind the meat firmly to produce a smooth sausage. Furthermore, the inside coating being water-swelling will adhere well to the sausage meat and prevent the formation of unsightly air blisters between the casing and the meat.

One embodiment of the process of the invention is illustrated in Fig. 1, in which a paper strip 1 of suitable width is led from the roll 2 over a roll 3 which applies adhesive from a bath 4 in a narrow line adjacent one edge of the strip which is then folded into a tube with the overlapping edges forming a seam by means of a conventional tube-forming machine 5. The tube 6 is passed under a roll 7 which applies a hardening agent from the hopper 8 to the seam. If necessary the tube may be passed through a drying chamber 9 to dry the adhesive. The seamed tube now may be wound up into a roll or passed immediately into a bath 10 containing the film-forming substance in suitable solvent, the tubing passing vertically from this bath into a heated chamber 11 which serves to dry and/or harden the film-forming substance. A quantity of the film-forming solution may be maintained inside the tube as shown. Preferably the tube is inflated as by trapping a volume of air between the solution and the roll 12. From the drying chamber 11, the coated and/or impregnated tube may be passed directly to the wind-up reel 13 but is preferably passed into a bath 14 containing a suitable liquid to further harden and insolubilize the film-forming substance. This bath may also contain a softening agent for the film-forming substance. From the bath 14, the tube passes to a drying chamber 15 wherein the tube is dried preferably in an inflated condition as by trapping a volume of air between the pairs of rollers 16 and 17 as shown. After drying, the tube may be wound on the reel 18 or cut into suitable sections for use as sausage casings. The product is shown in Fig. 2 and comprises a tube 6 having a longitudinal seam 19 secured by a layer of adhesive 20, the tube being coated on the interior and exterior with a continuous film 28.

It is important that the paper tubing be formed in such a manner that the seam does not lie on the folded edge of the tubing when it is wound up but lies, as nearly as possible, in the center of the flat side of the tubing. This gives a more uniform coating over the seam when the tubing is subsequently passed through the film-forming solution and this, of course, vitally strengthens the seam.

The treatment of the tubing with the film-forming solution may be effected in such a manner that the tubing is passed, in a flattened condition, through the film-forming solution, the time of treatment being so regulated that the solution penetrates sufficiently into the paper. The excess solution that is carried along on the strip may be wiped off by doctor blades. The use 75 of doctor blades involves certain difficulties in

maintaining a uniform wall thickness; therefore, it is desirable to eliminate the use of such scrapers. This is achieved, according to the invention, by using a film-forming solution of such a degree of viscosity and by drawing the paper tube, as it leaves the solution, vertically upwards at such a rate of speed that, on the one hand, the solution penetrates the paper with the degree of uniformity desired and, on the other hand, no more of the solution is carried along by the tubing than is required to obtain the desired wall thickness.

To produce a uniformly thick coating both inside and outside, the impregnated and coated tubing is preferably inflated before it leaves the film-forming solution, whereby there is obtained uniform impregnation and/or a uniform wall thickness in the finished artificial casing. The viscosity of the coating solution may be widely modified by the selection of the original components and by the concentration and temperature.

It is advisable to use an albuminous (protein) substance, e. g., a gelatine which, while having not too high a viscosity of its own, has as low as possible a degree of decomposition. With such 26 solutions, tubing is obtained which while the wall thickness is no greater, has a very high tensile strength, not inferior to that of natural casings.

Since albuminous solutions, as a result of their surface tension, easily tend to form foam, whereby defective spots occur on the casing when it is passed through the solution, certain foam-inhibiting substances preferably are added to the coating solution as in the bath 10. Suitable substances for this purpose are, for example, alcohols, such as ethanol, butanol, propanol and the like.

When the film-forming substance is initially a water-soluble substance such as gelatine, it is essential to subject the tubing after it has been 40 coated to a hardening process, e. g., with a formaldehyde solution as in bath 14, or with formaldehyde vapor which may be supplied to the chamber 11. Preferably the tubing is treated on the outside only with the hardening agent, as it is desirable that the inside coating remain unhardened so that the casing may better adhere to the sausage meat. To obtain casings having a good feel and a substantial flexibility, one may add to the formaldehyde solution in bath 14 a softening agent, such as glycerine.

By way of illustrating, but not by way of limiting the invention, the following example will be given:

A long fibred paper having a weight of 40 grams per square meter is conveyed from a supply roll to a tube-making machine wherein the edges are united by means of a 20% aqueous solution of a strong animal glue. The seam thus formed is saturated with a 5% aqueous solution of formaldehyde and dried for a short time. The paper tubing so constructed is then passed through a solution comprising:

|                                                                                | Grs. |
|--------------------------------------------------------------------------------|------|
| Gelatine having a viscosity of 170 seconds at 75° C. (by the method of Engler) | 66   |
| Water                                                                          | 150  |
| Alcohol                                                                        | 770  |
|                                                                                | 80   |

The temperature of this solution is kept constant at 75° C. The speed with which the paper tubing passes through the solution is approximately 6 meters per minute. From the coated end air is blown into the tubing until its cross-section is substantially circular. The tubing is dried for 75

a short time at an elevated temperature, then the gelatine coating hardened on the outside only by passing the tubing through a solution comprising:

|                   | Grs. |
|-------------------|------|
| Formaldehyde..... | 40   |
| Glycerine.....    | 100  |
| Water.....        | 860  |

10 and finally dried at an elevated temperature while inflated.

The finished casing has to a high degree the desirable properties of natural gut, in strength, elasticity, flexibility, pliability and porosity, and 15 like natural animal membranes, possesses the unique property of high expansion in the moistened condition and contraction when dried. It has also been found to satisfactorily meet the exacting requirements of casings when smoking, 20 curing and boiling processes are involved.

The product of this invention, therefore, is especially practicable for use in a tubular or other shaped container for foods intended for human consumption, although it is to be understood 25 that it may be used for receiving and preserving substances of a non-edible nature, or, in fact, wherever and whenever a container or casing with the properties of natural casing is required.

We claim:

30 1. In a process for making artificial sausage casings, the steps comprising forming a sheet of fibrous material into a tubing, forming a seam therein by uniting the overlapping edges of the sheet with a water-insoluble, non-swelling adhesive applied directly to the fibrous material and thereafter passing the tubing through a solution of a water-swelling, film-forming material with the interior and exterior surfaces of the tubing in contact with the solution and inflating 35 the tubing as it passes out of said solution.

40 2. In a process for making artificial sausage casings, the steps comprising continuously forming a sheet of paper into a tubing having the longitudinal edges overlapping, sealing said overlapping edges with a gelatine adhesive, insolubilizing the gelatine adhesive in the seam, passing the tubing so formed through a solution of gelatine with the interior and exterior surfaces of the tubing in contact with the gelatine, withdrawing the tubing from the solution in a vertical direction while inflating the tubing, thereafter insolubilizing the gelatine coating on the exterior and drying the coated tubing.

45 3. In a process for making artificial sausage

casings, the steps comprising treating tubing formed of a paper sheet having a seam formed with a hydrophobic colloidal adhesive with a solution of a hydrophilic film-forming material on the interior and exterior surfaces and withdrawing the tubing from said solution in a vertical direction while inflating the tubing, the rate of withdrawal being correlated with the viscosity of the solution so as to give a uniform coating of the desired thickness.

5 4. As an article of manufacture, an artificial sausage casing comprising a tubing formed of a sheet of paper having a longitudinal seam therein formed with a hydrophobic colloidal adhesive and coated on the interior and exterior with a 15 hydrophilic film-forming material.

5 5. As an article of manufacture, an artificial sausage casing comprising a tubing formed of a sheet of fibrous material having a seam formed with an insolubilized gelatine adhesive, the tubing being coated on the interior and exterior 20 with a film of gelatine which has been partially insolubilized substantially on the exterior of the tubing.

6 6. A process for making artificial sausage cas- 25 ing comprising forming a sheet of fibrous material into a tubing with longitudinal edges of the sheet overlapping, sealing the overlapping edges together with a water-insoluble adhesive, coating the interior and exterior surfaces of the tubing 30 with a water-swelling, film-forming material, and treating the exterior coating with a hardening agent.

7. A process for making artificial sausage cas- 35 ing comprising forming a sheet of fibrous mate- 35 rial into a tubing with longitudinal edges of the sheet overlapping, sealing the overlapping edges together with a water-insoluble adhesive, coating the interior and exterior surfaces of the tubing with a water soluble, film-forming material, and 40 treating the exterior coating with a solution containing a substance to render the coating insoluble in water and another substance to render the coating soft and flexible.

8. An artificial sausage casing comprising a 45 tubing formed of a sheet of fibrous material having the edges of the sheet overlapping to form a seam, an insolubilized gelatine adhesive sealing the overlapping edges together, a coating of soft gelatine on the interior of the tubing, and a 50 coating of a hardened, water-insoluble gelatine on the exterior of the tubing.

RICHARD WEINGAND,  
GUNTHER BRUNNEMACK